

# UNITED STATES PATENT OFFICE.

BRUNO MARIA ERNST LORENZ POSSANNER VON EHRENTHAL, OF CÖTHEN, GERMANY,  
ASSIGNOR OF FORTY-FIVE ONE-HUNDREDTHS TO MAX VON HALLE, OF HAMBURG,  
GERMANY.

## METHOD OF PRODUCING CELLULOSE AND OTHER PRODUCTS.

1,153,834.

Specification of Letters Patent. Patented Sept. 14, 1915.

No Drawing.

Application filed January 19, 1914. Serial No. 813,126.

To all whom it may concern:

Be it known that I, BRUNO MARIA ERNST LORENZ POSSANNER VON EHRENTHAL, of Cöthen, of the Dukedom of Anhalt, in Germany, have invented a new Method of Producing Cellulose and other Products, of which the following is the specification.

There are quite a series of vegetable fibers, which contain good fibers suitable for making paper, which however on account of the chemical construction are very difficult to be opened out and which heretofore could not be turned into bleachable cellulose in an economical manner. The reason of this is to be found in the chemical composition of these fibers so difficult to be opened out differing from the common raw cellulose material, such fibers containing usually larger amounts of low carbohydrates easily hydrogenized, moreover pectin substances and hemicelluloses and so on, which are all decomposed when alkaline opening out is resorted to and result in yellow to dark brown products, that cannot be washed out from the fibers and cannot be bleached or at least extremely difficult by the usual means. On the other hand those fibers, which are difficult to be opened out, will even withstand an acid opening out by the usual sulfite method because they are frequently strongly silicified and always contain an abundant amount of resin and gummy substances and also lignin substances, so that even by the aid of the acid boiling processes only a partial opening out is obtained while at the same time cellulins are produced which cannot be bleached at all or with great difficulty.

The object of the present invention is to overcome these difficulties which is done by submitting such fibrous substances difficult to be opened out to a combined acid and alkaline treatment. The fibrous substances are first subjected to the action of sulfite liquor in one of the usual pressure boilers. This method differs from the usual sulfite methods inasmuch as the composition of the methods lye must be different. The usual sulfite solutions contain about 1% CaO(MgO) and 4-5% SO<sub>2</sub> with a proportion between the free and the combined acid of about 2:1. When such fibrous substances difficult to be opened out are boiled with solutions of the said description a substance is obtained,

which, it is true, is soft but which is brown and unbleachable on account of the fact, that in such fibrous substances a greater amount of acid organic combinations of sulfurous acids (sulfon or sulfin acids) which are not fully combined by the small amounts of bases (lime, magnesium) and bring about the browning. To avoid this according to the present invention a solution is employed, which on account of a greater percentage of bases prevent the creation of such organic free acids. The liquor is saturated with bases as much as possible without precipitating monosulfite which is difficult to dissolve, according to the percentage say for instance 3-4% CaO at 4-5% SO<sub>2</sub>. At a maximum pressure of about 5-6 atmospheres and a maximum temperature of 125-130° C. a boiling of 6-7 hours will be sufficient to open out the fibers to such an extent to make them suitable for further efficacious treatment. The fibrous substances boiled with sulfite liquor will be subjected to a mechanical disintegrating process in a known manner followed by a thorough washing operation. The intermediate and the final liquor obtained by the sulfite boiling are to be worked in a known manner into sulfurous acid and on the other hand the organic substance dissolved therein, not having undergone such an extensive destruction on account of the weak boiling, will be recovered by neutralization and precipitation or by evaporation to a form fit for use or will be treated in a known manner for producing alcohol.

The fibrous material gained by the sulfite boiling process which even when washed, still will have a more or less brown color and also contains numerous organic combinations difficult to be bleached is for the purpose of a further opening out heated together with a 5-10% solution of calcined soda or still better of caustic soda in open vessels (preferably in a bleaching engine) to 80-90° C. and then digested one or more hours according to the condition of the fibrous materials. This is done according to the counter current principle so that the fresh soda solution comes into contact with fibers that are pretty well lixiviated while the liquor which is enriched with organic substances is brought into contact with the mass not yet digested with any alkaline liquor, so that the liquor is saturated with or-

ganic substance as much as possible. In the same manner the substance is hereafter washed with cold or hot water according to the counter current principle, the washing water saturated with alkali can be used also for the alkaline digestion. By such alkaline treatment the organic combinations that are difficult to bleach are dissolved out from the mass, so that the fibers thus purified can easily be bleached by the usual bleaching means.

The organic substances contained in the alkaline solution consists mainly of vegetable proteins, fatty matters as well as gum- and resin-substances and can easily be extracted by neutralizing the liquor with mineral acids in a powdery form while the dissolved silicates are not precipitated. For the purpose of neutralization sulfuric acid or sulfurous acid will be most advantageous since by the same the organic substances will be precipitated to the greatest extent. When the organic substance has settled the solution of sulfate or sulfite of soda respectively will be poured off, and may be returned into the cycle of operation or after having been first rendered alkaline with caustic lime. If sulfurous acid is used for neutralization the calcium monosulfite which is formed by rendering the solution alkaline and which is difficult to dissolve can also be returned into the cycle of operation for the preparation of the fresh sulfite solution. The precipitated organic substance may according to its chemical condition be used as an animal food when drained and dried (an analysis resulted in for instance with bagasse 5.25% protein, 3.30% fatty matters, no silicic acid, no ashes) and can also be

used for producing glue and other adhesives.

I claim:

1. In the method of producing cellulose and other products, the step which comprises boiling the fibrous material with a weak acid sulfite liquor at a pressure of from 5-6 atmospheres and a temperature not exceeding 125°-130° C., then mechanically disintegrating and washing the substance, digesting it with soda at increased temperature, and finally washing it out.

2. In the method of producing cellulose and other products, the step which comprises boiling the fibrous material with a weak acid sulfite liquor at a pressure of from 5-6 atmospheres and a temperature not exceeding 125°-130° C., then mechanically disintegrating and washing the substance, digesting it with caustic soda at increased temperature and atmospheric pressure, and finally washing it out.

3. In the method of producing cellulose, the step, which comprises boiling fibrous material with a sulfite liquor weak in acid and containing a base just short of sufficient to precipitate said base as monosulfite, said boiling being under a pressure of from 5-6 atmospheres and at a temperature not exceeding 125°-130° C., then mechanically separating the fibers and finally digesting them with soda at an elevated temperature and normal atmospheric pressure.

BRUNO MARIA ERNST LORENZ  
POSSANNER VON EHRENTHAL.

Witnesses:

F. A. MAX KAEMPF,  
ERNEST H. L. MUMMENHOFF.